

(No Model.)

R. R. WAITZ.

PROCESS OF PREPARING REFRACTORY ORES FOR AMALGAMATION.

No. 247,972.

Patented Oct. 4, 1881.



Witnesses:

All Long  
A. M. Tanner

Inventor.

Robert R. Waitz.

By Paine, Chaffton & Ladd

Attorneys.

# UNITED STATES PATENT OFFICE.

ROBERT R. WAITZ, OF ROSITA, COLORADO.

## PROCESS OF PREPARING REFRACtORY ORES FOR AMALGAMATION.

SPECIFICATION forming part of Letters Patent No. 247,972, dated October 4, 1881.

Application filed September 9, 1881. (No model.)

*To all whom it may concern:*

Be it known that I, ROBERT R. WAITZ, a citizen of the United States, residing at Rosita, in the county of Custer and State of Colorado, have invented certain new and useful Improvements in Processes of Preparing Refractory Ores for Amalgamating; and I do hereby declare the following to be a full, clear, and exact description of the invention, such as will enable others skilled in the art to which it appertains to make and use the same, reference being had to the accompanying drawing, and to letters or figures of reference marked thereon, which form a part of this specification.

The object of my invention is to furnish a process for treating refractory auriferous and argentiferous ores, by means of which the base metals contained in said ores are thoroughly and quickly converted into insoluble oxides, and all volatile matters decomposed and expelled from the furnace. I attain the results stated by heating the pulverized ore in a scientific manner in a furnace or chamber from which atmospheric air is excluded, as will hereinafter be more fully set forth, and then indicated in the claim.

In carrying out my process I pulverize or comminute the ore containing the precious metals, and add thereto, before or after its introduction into a furnace or heating-chamber, any well-known oxygenated agent or substance—such as dioxide of manganese, chloride of potassium, or ferric oxide. These substances may be used singly, or two of the same or all three may be combined. The proportions in which they are used depends altogether upon circumstances or the character of the ores, because the latter frequently contain the aforesaid substances. It is an essential requisite that no sulphates shall be present in the ore when the same is undergoing the process of amalgamation, and for this reason I also add to the ore, before or after its introduction into the furnace, an agent or substance which will serve to decompose the sulphates formed—particularly sulphate of copper. In certain instances the carbonic-acid gas evolved by the combustion of fuel in the fire-chamber of the furnace will serve to accomplish the result stated. When copper pyrites are being

treated I preferably add thereto a sufficient quantity of the well-known reagent—carbonate of ammonium—for decomposing sulphates. In this instance the latter are converted into volatile sulphate of ammonia, which passes off. 55

It has already been stated that the invention consists chiefly in a scientific manner of heating the ores, and I will now proceed to fully describe the same, reference being had to the accompanying drawing, which illustrates a furnace preferably employed for carrying out my process.

The pulverized ore is fed into a closed flue or chamber, and is conducted or passed through the same in the form of a thin stratum or body, which is in constant motion from the inlet to the outlet openings. In the form of furnace illustrated in the drawing the ore moves by its own gravity through an inclined flue or chamber, and is discharged upon a horizontal hearth or sole located in juxtaposition to the grate or fire chamber. It will be manifest, however, that the ore can be moved by mechanical means through a horizontal flue or chamber. The flames and heated gases issuing from the fire or grate chamber pass through the flue or ore-treating chamber and obviously cause an excess of oxygen to evolve from the oxygenated substances contained in the ore. The thin stratum or body of ore will enable this result to take place in an expeditious and perfect manner, because the sheet of flame is brought into intimate contact with the ore. 75

It is necessary to the proper heating or roasting of ores that the same be heated gradually, 85 so as to obviate the fusion of sulphides at the outset and prevent the formation of a matte troublesome to roast. In my process the action of the heat is, as just stated, because the ore is constantly moving from the feed-hopper 90 farthest from the fire-chamber to the discharge-passage in proximity to the latter.

The liberation of oxygen by heat in the manner above indicated will not only serve to effect the perfect oxidation of the base metals 95 without the aid of an air-blast or current of atmospheric air, but will also tend to supply the necessary amount of oxygen to the fire-chamber for supporting the combustion of fuel therein.

It will be obvious that the descending or moving body of ore will effect a back action of the oxygen existing near the fire-chamber, and force the same into the latter; hence it is possible to support combustion with closed furnace-doors, there being no admission whatever of atmospheric air.

- 5 My process is specially designed for treating refractory ores of precious metals, because I am able to perform the heating operation with a small consumption of fuel and in a comparatively brief period of time—one to two hours. The roasted ore passing from the furnace contains the precious metals in a pure 15 metallic state, and as all base metals have been converted into insoluble oxides and the sulphates decomposed, the process of amalgamation with mercury can be performed in a thorough and expeditious manner.
- 20 I am aware that it is not new to add oxygenated substances to ores while undergoing the roasting operation in a furnace having means for admitting atmospheric air, and devoid of devices for propelling the ore. It has 25 also been proposed to roast ores, mixed with oxygenated agents, in a retort or closed cylinder revolving in a fire-chamber, and having a steam-jet pipe leading into said retort.
- I am also aware that ore has been passed 30 through a flue or roasting-chamber in the form of a thin stream or stratum moving constantly from inlet to outlet, and subjected to the ex-

idizing action of a current of atmospheric air and heated gases.

I disclaim the various steps of my process, 35 separately considered, and confine myself to the combination of steps herein set forth, which promise a success much surer and a roasting far better and expeditious than by any other process heretofore proposed.

Having thus described my invention, what I claim as new, and desire to secure by Letters Patent, is—

The process of desulphurizing and oxidizing refractory auriferous and argentiferous ores, 45 consisting in subjecting a thin body or stratum of ore, moving constantly through a closed chamber from which air is excluded, to the direct contact of a caloric current or sheet of flame, and of oxygen, evolved by the decom- 50 position of oxygenated agents contained in the ore, through the medium of heat, the oxygen so obtained, in addition to its oxidizing action, serving to support combustion in the ore-chamber, and in a fire-chamber communicating directly with the latter, substantially as set forth.

In testimony whereof I affix my signature in presence of two witnesses.

ROBERT R. WAITZ.

Witnesses:

EUGENE D. CARUSI,  
W. B. T. KEYSER.